

## UNITED STATES PATENT OFFICE

1,987,213

## MANUFACTURE OF WATER-LAID FELTS

George A. Richter, Berlin, N. H., assignor to  
 Brown Company, Berlin, N. H., a corporation  
 of Maine

No Drawing. Application December 10, 1932,  
 Serial No. 646,740

12 Claims. (Cl. 92—3)

This invention relates to the manufacture of absorptive papers or water-laid felts designed more particularly for impregnation purposes.

In the manufacture of impregnated sheet products, it is sometimes the practice to use as the base sheet one which has been felted on machinery of the paper-making type. While various kinds of fibrous material may be employed as the felt-making furnish, it has heretofore been the practice in some industries, notably the roofing and floor-covering industries, to use as the raw material, waste rags of various descriptions. These rags are conditioned for the felt-making operation in a so-called hollander or beater engine, wherein they are beaten in the presence of water for the purpose of disintegrating the pieces of cloth until there is produced a pulp or half-stuff made up of fibers whose size is such as to permit their felting on a paper-making machine into a sheet of uniform texture. In some instances, the raw rags, as they are purchased on the open market, are subjected to a purifying or cleansing treatment in dilute alkaline solutions at elevated temperatures and are then washed free of the solution, before they are subjected to beater action. In any case, however, the beating or reduction of the rags in water to form a pulp or half-stuff is accompanied by a hydration of the cellulose fiber. While such hydration may be desired in those instances where papers of high strength and tear resistance are desired, nevertheless, it has been my observation that hydration is an undesirable factor when felts designed for impregnation purposes are in question. Indeed, the hydrated cellulose tends to reduce the absorptivity, softness, and flexibility of the felt, even though it enhances such physical qualities as strength and tear resistance.

In accordance with the present invention, therefore, the reduction of rags in water to form a pulp or half-stuff suitable for the felt-making operation on a paper-making machine is accomplished while preserving the pulp in a substantially unhydrated or "free" state. This result is had by converting the raw rag stock into a substantially non-hydratable state before it is subjected to reduction or disintegration in water in a beater engine, wherefore, hydration or gelatinization of the stock is inhibited during the beating operation and the resulting pulp or half-stuff can be formed into water-laid felts characterized by their high absorptivity, softness, and flexibility. Despite the fact that felts so made may initially be tender and lacking in much tensile strength or tear resistance, they can be impregnated quickly and uniformly with various binders, such as latex, natural and synthetic resins, cellulose ester solutions, waxes, bitumen, or other binders of a thermoplastic, water-dispersed, or dissolved variety, to form impregnated products of a high binder content and characterized by a highly desirable combination of characteristics. The felt may, for example, be bituminized to form a sheet which is highly pliant and practically proof against tear, especially the initiation of tear. Apparently, the fact that the contiguous fibers in the sheet are not bonded strongly by hydrated cellulose is responsible for the high tear resistance in the bituminized sheet, since it is quite likely that when a tearing stress is applied to the sheet, the stress, rather than becoming localized and giving rise to rupture of the sheet, is not confined to any particular locus, but is distributed and/or dissipated over a large area on account of the freedom of the fibers to slip or move past one another.

While various chemical reagents may be used to convert the raw rag stock to a substantially non-hydratable state, I have found that a most effective and practical way of accomplishing this result is to subject the rag stock to the action of mercerizing liquors for a sufficient period of time to mercerize the cellulose and thereby make it non-hydratable. In using the term "mercerize", I mean that the stock undergoes the action of a caustic soda solution whose activity is preferably that of a caustic soda solution of at least about 18% strength at room temperature, although the term is meant to embrace the use of solutions whose activity corresponds to a caustic soda solution of about 10% strength at room temperature, as such latter solutions, while they do not mercerize to completion, nevertheless change the cellulose fiber structure so as to make it difficultly hydratable. An important advantage gained through the use of a mercerizing liquor, besides that of transforming the cellulose to a non-hydratable state, is that it functions as a cleansing or purifying agent, tending to dissolve degraded cellulose, and other impurities foreign to or inherent in rag stock.

A specific treatment to be applied in accordance with my invention to rag stock may involve mixing of the rag stock as it is purchased on the open market with a solution of caustic soda of about 18% or greater strength at room or below room temperature. The rags may be mixed with sufficient solution, say, about 10 or more parts by weight of solution to 1 part by weight of dry rags, to ensure sufficient liquor to cover or sub-

merse the rags, and the mixture may be gently stirred over a period of, say, 30 minutes to 6 hours. Under such conditions, the rag stock becomes mercerized and purified, the extent of 5 mercerization and purification depending upon the duration of the treatment. After the treatment, the mercerizing liquor may be separated from the rag stock, as in a counter-current washer designed to effect washing of the stock 10 with minimum dilution of the liquor so that the liquor may be re-used in the treatment of other raw rag stock. If desired, rather than washing the stock free from mercerizing liquor, the excess liquor may be separated without dilution as in a 15 centrifuge, thickener, or other filtering or separating apparatus. A portion of the liquor, in fact, most of the liquor, may thus be recovered in an undiluted condition and be re-used with little, if any, fortification in the treatment of other raw 20 rag stock. The centrifuged or thickened rag stock may then be washed free of the residual mercerizing liquor as hereinbefore described.

When the rag stock is treated at temperatures below normal or room temperature, the causticity 25 of the liquor requisite for the mercerization of the stock may be lower than the 18% caustic soda solution which mercerizes at room temperature. It is well known that mercerization is promoted by the lowering of temperature and that 30 the lower temperature, the lower the concentration of the caustic soda solution requisite for mercerization. Consequently, when the rag stock is treated with a refrigerated caustic soda solution, for instance, one at 0° to 5° C., mercerization 35 may be effected with a caustic soda solution containing as little as about 5% caustic soda. It is, in fact, possible to operate at temperatures below the freezing point, in which case, mercerization may be effected with even more dilute caustic 40 soda solution, as in such case, ice or water crystals separate out from the solution, in consequence of which the unfrozen or liquid portion of the solution becomes more concentrated in caustic soda and functions more effectively as a mercerizing 45 agent. In the event that the treatment of the rag stock is performed with a refrigerated or partially frozen mercerizing liquor, it is of decided advantage to separate out the excess refrigerated liquor from the stock so as to conserve 50 it in a refrigerated as well as undiluted condition for the treatment of other raw rag stock. Should a portion of the mercerizing liquor be frozen, it may be thawed out to permit a separation of as much liquor as possible from the stock, 55 before the stock is washed.

The alkaline liquor used for the purpose of the present invention may, if desired, contain alkalies other than caustic soda, for instance, sodium sulphide. Thus, the so-called white liquor of a 60 kraft pulp mill, which, as is well known, contains sodium sulphide as well as caustic soda, may be employed under mercerizing conditions, as hereinbefore defined. So, too, the mercerizing liquor may contain suitable oxidants, such as hypo- 65 chlorite bleach, sodium peroxide, hydrogen peroxide, permanganate, or the like. An oxidant should not, however, be used in the mercerizing liquor when a reducing agent like sodium sulphide is present therein. A mercerizing liquor 70 containing an oxidant is of value more particularly in connection with colored rag stock, as it makes possible partial or complete decolorization of the rags, so that the halfstuff or pulp subsequently produced therefrom may be fabricated 75 into felts of lighter color, when such latter

quality is a desideratum. The fact is, that in some cases it may be advantageous to treat the rags with oxidants such as chlorine, hypochlorite bleach, permanganate, or the like, and then to wash the rags before they are treated in a mercerizing liquor containing, if desired, additional oxidant.

The washed, mercerized rag stock prepared as hereinbefore described may be charged into a hollander or beater engine together with sufficient water to ensure circulation and then reduced or beaten by the operation of the engine into a pulp or halfstuff fit for delivery to a felt-making machine. Inasmuch as the mercerized rag stock is practically non-hydratable, beating does not 10 tend to develop hydrated or gelatinized cellulose therein so that the finished pulp or halfstuff is in a comparatively "free" condition. The resulting felts reflect the freeness of the pulp furnish from which they have been prepared in that they are comparatively tender or lacking in tensile strength and tear resistance and in that they are highly porous, bibulous, soft and flexible. When impregnated with binders, however, these felts acquire enormous toughness, 15 strength and tear resistance. For instance, they become leatherlike in their properties when they are impregnated with rubber latex, rubber solutions or the like, and are then dried. They become tough, pliant, and practically tear-proof 20 when they are impregnated with bitumen or similar binders in the production of roofing and floor-covering materials.

In making the water-laid felts or foundations 25 of the present invention, it may be of advantage 30 to admix with the substantially unhydrated rag pulp or halfstuff, a suitable proportion of un- 35 mercerized cellulose pulp which may be in a sub- 40 stantially unhydrated, partially hydrated, or well-hydrated condition. The well-hydrated 45 pulp blended with the mercerized rag pulp or halfstuff may be prepared by overbeating rag 50 stock or other suitable cellulose fiber in much 55 the same way as is done in connection with the manufacture of glassine papers. The best kinds 60 of hydrated or gelatinized celluloses for blending with the mercerized rag pulp or halfstuff are 65 those prepared in a so-called stone-roll beater from kraft or other wood pulps which have been 70 refined by alkali to higher alpha cellulose content. The use of some unmercerized pulp facilitates 75 the production of uniformly-textured felts, serving to offset the clumping or bunching tendencies in mercerized pulp. It is, however, pos- 80 sible to avoid clumpy or non-uniform felt forma- 85 tion even when the entire felt-making furnish is 90 mercerized by delivering the furnish in an ex- 95 tremely dilute and well-mixed condition to the 100 felt-forming machine. The use of hot water as 105 a suspending medium for the felt-making furn- 110 ish also mitigates the clumping or bunching 115 tendencies of the mercerized fibers.

Since the present invention is centered about 120 the use of rag stock as a felt-making raw mate- 125 rial, it is well to define what I mean by rag 130 stock. In using the expressions "rags" or "rag 135 stock", I mean cellulose fiber occurring in the 140 form of woven and/or knitted fabric or strand 145 material such as cloth, burlap, rope, or the like, 150 made up of cotton, linen, jute, or similar cel- 155 lulose fiber yarns which must be disintegrated or 160 reduced to form a comparatively short-fibered 165 pulp or halfstuff before satisfactory formation 170 into felts can be realized on machinery of the 175 paper-making type. In some instances, the rags

may contain non-cellulosic fibers, such as wool and/or silk, but inasmuch as these are largely dissolved or destroyed by mercerizing solutions, it is preferable to work with rags consisting 5 practically in entirety of cellulose fibers. Waste rags containing artificial silk, such as viscose-rayon, can be used, for artificial silk is not wholly destroyed by mercerizing solutions.

It is to be observed that in accordance with 10 my invention, practically no beating of the rags is performed before the rags are mercerized and the mercerizing liquor is washed therefrom. While my entire process, including mercerization and washing, might be performed in a beater engine, nevertheless, during the initial stages of the 15 process, that is, before the stock has been mercerized to a non-hydratable condition, the beater roll should not be operated to beat or reduce the stock but merely to effect circulation and mixing; otherwise, considerable cellulose would be 20 lost on account of initial hydrating tendencies and the loss of the hydrated cellulose in the mercerizing liquor. It is only after the stock has become substantially non-hydratable that I 25 lower the beater roll to effect a cutting or reducing action of any moment. Indeed, I prefer to effect such beating or reducing action after the mercerizing liquor has been substantially completely removed or washed from the stock.

30 Another important advantage inhering in my invention is that when rag stock is treated with strong alkaline liquor substantially without disintegration or reduction of the rags into fibers or fiber fragments, the recovery of the unused alkali is facilitated because it is much easier to 35 remove the alkaline liquor from rags, as hereinbefore described, than from a mass of fibers or pulp dispersed in an alkaline liquor.

I claim:

40 1. A process which comprises converting rags to a substantially non-hydratable condition substantially without disintegrating or reducing them, and then mechanically reducing the non-hydratable rags in water to form a substantially ungelatinized pulp or halfstuff consisting of fibers feltable into a uniform texture.

2. A process which comprises treating rags with a mercerizing liquor substantially without disintegrating or reducing them, thereby converting them into a mercerized, substantially non-hydratable condition, and beating the rags in water to form a substantially ungelatinized pulp or halfstuff consisting of fibers feltable into a uniform texture.

55 3. A process which comprises converting rags to a substantially non-hydratable condition substantially without disintegrating or mechanically reducing them, reducing the non-hydratable rags in water to form a substantially ungelatinized pulp or halfstuff consisting of fibers feltable into a uniform texture, and forming such pulp or halfstuff into a water-laid felt.

4. A process which comprises treating rags with a mercerizing liquor substantially without disintegrating or reducing them, thereby converting them into a mercerized, substantially non-hydratable condition, beating the rags in water to form a substantially ungelatinized pulp or halfstuff consisting of fibers feltable into a uniform texture, and forming such pulp or halfstuff into a water-laid felt.

5. A process which comprises treating rags with a mercerizing liquor substantially without disintegrating or reducing them, thereby converting them into a mercerized, substantially non-hydratable condition, removing the mercerizing liquor from the rags, beating the rags in water to form a substantially ungelatinized pulp or halfstuff consisting of fibers feltable into a uniform texture, and forming such pulp or halfstuff into a water-laid felt.

10 6. A process which comprises treating rags with an oxidant, and then treating the rags with a mercerizing liquor containing an oxidant substantially without disintegrating or reducing them, thereby converting them into a mercerized, 15 substantially non-hydratable condition, and beating the rags in water to form a pulp or halfstuff consisting of fibers feltable into a uniform texture.

20 7. A process which comprises treating rags with a mercerizing liquor containing an oxidant substantially without disintegrating or reducing them, thereby converting them into a mercerized, substantially non-hydratable condition, and beating the rags in water to form a pulp or halfstuff 25 consisting of fibers feltable into a uniform texture.

25 8. A process which comprises treating rags with an oxidant, then treating them with a mercerizing liquor substantially without disintegrating or reducing them, thereby converting them into a mercerized, substantially non-hydratable condition, and beating the rags in water to form a pulp or halfstuff 30 consisting of fibers feltable into a uniform texture.

35 9. A process which comprises treating rags with a mercerizing liquor containing an oxidant substantially without disintegrating or reducing them, thereby converting them into a mercerized, substantially non-hydratable condition, beating the rags in water to form a pulp or halfstuff 40 consisting of fibers feltable into a uniform texture, and forming such pulp or halfstuff into a water-laid felt.

45 10. A process which comprises treating rags with a mercerizing liquor substantially without disintegrating or reducing them, thereby converting them into a mercerized, substantially non-hydratable condition, beating the rags in water to form a substantially ungelatinized but mercerized pulp or halfstuff 50 consisting of fibers feltable into a uniform texture, admixing unmercerized pulp with such mercerized pulp or halfstuff, and forming the mixture into a water-laid felt.

55 11. A process which comprises treating rags with a mercerizing liquor containing sodium sulphide while maintaining them in a substantially unreduced condition, and beating the resulting mercerized rags in water to form a substantially ungelatinized pulp consisting of fibers feltable into a uniform texture.

60 12. A process which comprises treating rags with a mercerizing liquor containing sodium sulphide while maintaining them in a substantially unreduced condition, beating the resulting mercerized rags in water to form a substantially ungelatinized pulp consisting of fibers feltable into a uniform texture, and forming such pulp into a water-laid felt.

70 GEORGE A. RICHTER.